

# UNITED STATES PATENT OFFICE.

JAMES C. PEABODY, OF BOSTON, MASSACHUSETTS.

## PROCESS OF MAKING PAPER, FIBER-BOARD, AND SIMILAR MATERIALS.

1,376,353.

Specification of Letters Patent. Patented Apr. 26, 1921.

No Drawing.

Application filed October 23, 1918. Serial No. 259,413.

*To all whom it may concern:*

Be it known that I, JAMES C. PEABODY, a citizen of the United States, residing at Boston, in the county of Suffolk and Commonwealth of Massachusetts, have invented certain new and useful Improvements in Processes of Making Paper, Fiber-Board, and Similar Materials, of which the following is a specification.

10 In the usual process of making paper, fiber board or similar materials, the stock, which consists mainly of a mass of fibers, is first beaten in a beater in the presence of water, and the resulting pulp is then run 15 into a stuff-chest from which it is drawn in a continuous stream into the vat or tank of the machine in which the paper or fiber board is to be formed, such machine being usually either of the cylinder or of the Four- 20 drinier type. The proportion of water to fibrous stock in the beater and in the stuff-chest is ordinarily considerably less than the proportion of water to fibrous material in the tank or vat from which the stock is supplied directly to the cylinder or Fourdrinier 25 machine. For example, a usual proportion of water to fiber in the beater and stuff-chest may be perhaps 20 pounds of water to one of fiber, whereas in the vat of the 30 cylinder machine a usual ratio of water to fiber may be perhaps 50 pounds of water to one of fiber. Accordingly, before starting the flow of stock from the stuff-chest into the vat of the machine, when operation of 35 the machine is to be begun, it is customary to place in the vat a quantity of water sufficient to increase the proportion of water to fibrous stock to the requisite degree.

In the manufacture of certain kinds of 40 paper, or fiber board, there is introduced into the stock in the beater, stuff-chest or other preliminary container, some added material which may be colloidal or cementitious in its nature, the amount which is so 45 added being such as to give a predetermined standard of concentration. When this stock of said standard of concentration is run into the tank or vat of the paper machine, a stock having a much lower standard 50 of concentration is produced owing to the dispersion in the fluid therein contained, and when the fiber is gathered by the machine, it contains much less than the desired proportion of the added substance, the balance

having run off in the waste water. This 55 method has two serious defects. In the first place, the product produced does not contain the intended proportion of the added substance and does not have the qualities which it should have, and in the second place, there 60 is a serious loss due to the waste of the added material which is carried off in the waste water. These defects are so serious that it has been thought to be impossible to 65 introduce certain substances by placing them in the beater, although in other respects better results are so obtained, and instead, attempts have been made to impregnate the product after it comes from the paper machine. This has proved wholly impracticable for reasons which need not be explained here.

My present invention, therefore, provides a method by which certain substances, some of which are colloidal, cementitious, or 75 soluble in their nature, may be mingled with the fiber in the beater, and the fiber may be gathered by a paper machine without loss of the added substance, the entire run of the machine being uniform in respect to the 80 proportion of the added substance.

Furthermore, I find that it is frequently possible to use a different added substance in the tank of the paper machine than in the preliminary container, particularly when 85 the substance is colloidal owing to the fact that colloidal substances are not interpenetrable.

While my herein described novel method is particularly applicable when the substance to be added is colloidal, I do not 90 limit myself to its use with such substances.

To make my method fully understood, I will describe the manner in which the manufacture of one kind of paper is actually performed. In the manufacture of this kind of paper, the added substance is an alkaline cellulose thiocarbonate, the function of which is to cement together the mass of fibers in the paper or board. I prefer to use this 100 material in my process, but may also use other substances in lieu thereof, such as glue, casein, or viscose.

According to my process, I may load a 105 beater with 250 pounds dry weight of a mixture of hemp, jute, wood or other fibers, 5,000 pounds of water, sizing material, coloring matter in any usual proportions, and

25 pounds of alkaline cellulose thiocarbonate. After the stock has been thoroughly beaten in the usual manner and the several ingredients properly incorporated throughout the mass of fibers, the beater load is discharged into the stuff-chest, where it may perhaps be mingled with comparatively small additional quantities of water.

10 I now fill the vat of my cylinder machine with water, say, 2,400 pounds.

It will be observed that the proportion of the alkaline cellulose thiocarbonate to water in the stock in the beater, in the instance illustrated, will be 200 pounds of water to 15 1 pound of thiocarbonate. The proportion of water to thiocarbonate in the stock in the stuff-chest, though perhaps somewhat larger, will not differ very materially. If, now, I begin to discharge the stock from 20 the stuff-chest into the vat of the cylinder machine and begin to operate the machine, during the first part of the run the proportion of water to thiocarbonate in the tank will be very much greater because of the 25 large amount of water in the tank which the stock meets and in which it is dispersed as it enters the tank.

I have found that the presence of this great excess of water in proportion to thiocarbonate in the tank during the early part 30 of the run makes it difficult to retain the thiocarbonate upon the fibers as they pass from the vat upon the screen and are taken away to form the finished board; and the 35 result is that the first part of the run of the board is very inferior in quality, because of the lack of these cementitious materials.

I have found that this difficulty may be remedied by adding to the water in the tank 40 of the machine a colloidal substance, such, for example, as alkaline cellulose thiocarbonate, glue, casein or viscose. I prefer to put into the water in the tank a sufficient quantity of such colloidal substance so that 45 the water will be brought to the same degree of concentration as the water in the stuff-chest. For example, in the illustrative run above mentioned, I should prefer to put into the 2,400 pounds of water in the vat 50 of the cylinder machine about 10 or 12 pounds of colloidal substance. While I prefer to bring the water in the tank of the machine to substantially the same degree of concentration as the water in the stuff-chest, nevertheless good results may be obtained by using less or greater quantities of 55 colloidal substance in the tank; and my invention is not limited to these proportions.

I also prefer to use as my colloidal substance in the tank the same material that is 60 used in the beater to give the cementitious effect. For example, if I use alkaline cellulose thiocarbonate in the beater I prefer to use alkaline cellulose thiocarbonate in the 65 water in the tank, and if I use glue in the

beater I prefer to use glue in the tank; but this is not necessary, and it is perfectly possible to use glue, for example, in the tank when thiocarbonate is used in the beater, or vice versa.

70

By this method of operation I find that the cementitious material in the stock as it comes from the stuff-chest is not washed out or dissipated when the stock enters the tank of the machine, but adheres to the fibers 75 as they pass from the tank upon the screen and appears in the finished product, where it acts to cement the fibers together.

Sometimes it is desirable to add additional water to the stock as it leaves the 80 stuff-chest or to the tank during the operation of the machine; and although I do not find that the addition of this water interferes with the proper functioning of the materials, I prefer to use for this purpose, 85 instead of fresh water, water that has drained off from the cylinder or the felts of the machine, since this reused water contains some of the thiocarbonate or other cementitious materials originally incorporated in it. This reuse of the water draining 90 from the machine is not, however, essential to my invention.

If at any time during the operation of the machine the proportion of colloidal substance to water in the tank becomes less than the critical amount necessary to prevent the washing out of the cementitious material, and it is found that the cementitious material is not being retained upon the fibers as 95 they pass from the vat, I fortify the stock in the tank by adding further quantities of colloidal substance to bring it up to the requisite proportion.

The product manufactured in accordance 105 with my process is formed on the cylinder or Fourdrinier machine, or otherwise in any known manner, into sheets or other forms as desired.

What I claim as new and desire to secure 110 by Letters Patent is:—

1. The process of making paper which consists in introducing an added material to a mass of fibers suspended in water in a preliminary container to form a stock of a 115 predetermined standard of concentration with reference to the added material, and forming the paper by means of a machine in which the fiber stock is further diluted but is maintained at substantially the same 120 standard of concentration of added material.

2. The process of making paper which consists in producing in a preliminary container a stock composed of fibers suspended 125 in water, said stock containing an added material and being of a predetermined standard of concentration with reference to the added material, diluting said stock and introducing more added material to restore 130

the standard of concentration of said added material, and then forming the paper.

3. The process of making paper which consists in producing in a preliminary container a stock composed of fibers suspended in water, said stock containing an added material and being of a predetermined standard of concentration with reference to the added material, and forming the paper 10 by means of a machine in which the stock is diluted and in which the standard of concentration is maintained by the introduction of an added material which is different from that which is introduced in 15 the preliminary container.

4. The process of making a product of the character described which consists in adding a cementitious material to a mass of fibers in a preliminary container to form 20 a stock, adding a colloidal substance to the water in the tank into which the stock is run and from which it is supplied to a machine for forming the product, and then forming the product.

25 5. The process of making a product of the character described which consists in adding a colloidal material to a mass of fibers in a preliminary container to form a stock, adding a colloidal substance to the water in the 30 tank into which the stock is run and from which it is supplied to a machine for forming the product, and then forming the product.

6. The process of making a product of 35 the character described which consists in adding a cementitious material to a mass of fibers mingled with water in a preliminary container to form a stock, and adding a colloidal substance to the water in the 40 tank into which said stock is run and from which it is supplied to a machine for forming the product, the proportion of colloidal substance added to the water in the tank being substantially similar to the proportion 45 of cementitious material to water in the stock before it is run into the tank, and forming the product.

7. The process of making a product of the character described which consists in 50 adding alkaline cellulose thiocarbonate to a mass of fibers mingled with water in a preliminary container to form a stock, and adding alkaline cellulose thiocarbonate to the water in the tank into which the stock 55 is run and from which it is supplied to a

machine for forming the product, and then forming the product.

8. The process of making a product of the character described which consists in adding a colloidal substance to a mass of 60 fibers mingled with water in a preliminary container to form a stock, adding a similar colloidal substance to the water in the tank into which the stock is run and from which it is supplied to a machine for forming the 65 product, and forming the product.

9. The process of making a product of the character described which consists in adding a colloidal substance to a mass of fibers mingled with water in a preliminary 70 container to form a stock, adding a similar colloidal substance to the water in the tank into which the stock is run and from which it is supplied to a machine for forming the product, said colloidal substance being 75 added to the water in the tank in substantially similar proportion to that which the colloidal substance bears to the water in the stock previous to its being run into the tank, and forming the product.

80 10. The process of making a product of the character described which consists in adding a cementitious material to a mass of fibers mingled with water in a preliminary container to form a stock, adding a 85 colloidal substance to the water in the tank into which the stock is run and from which it is supplied to a machine for forming the product, returning to the tank from time to time water previously drained from the machine, and forming the product.

90 11. The process of making a product of the character described which consists in adding a cementitious material to a mass of fibers in a preliminary container to form 95 a stock, adding a colloidal substance to the water in the tank into which the stock is run and from which it is supplied to a machine for forming the product, and maintaining the proportion of colloidal substance to 100 water in said tank at a percentage sufficient to prevent the washing out of the cementitious material, and forming the product.

In witness whereof, I have hereunto set my hand in the presence of two witnesses.

JAMES C. PEABODY.

Witnesses:

HARRISON F. LYMAN,  
GEORGE C. ARVEDSON.